

## UNITED STATES PATENT OFFICE.

FREDERICK W. KARITZKY, OF GARWOOD, NEW JERSEY, ASSIGNOR TO HENRY E. NEWHALL, OF PLAINFIELD, NEW JERSEY.

## ALLOY AND METHOD.

No Drawing.

Application filed December 31, 1924. Serial No. 758,974.

*To all whom it may concern:*

Be it known that J. FREDERICK W. KARITZKY, a citizen of the United States, residing at Garwood, in the county of Union and State of New Jersey, have made certain new and useful Improvements in Alloys and Methods, of which the following is a specification.

My invention relates to an alloy and the method of making it.

My invention further relates to an alloy of zinc, aluminum and tin, which can be cast in metal molds, and also in sand molds, at reasonable casting temperatures, the resulting casting being strong and rigid and there being no material breakage due to shrinkage in the mold.

Care must be exercised that the alloy will not shrink to a material extent in the mold for this would result in breaking the casting in the mold. The melting point of the alloy must not be too high, for with a high melting point the alloy cannot be satisfactorily poured into the mold. The ingredients must be so proportioned that the resulting casting will not be too brittle, which would result in a weak casting. The ingredients must also be so proportioned that the resulting casting will be rigid and strong.

The melting point of commercial aluminum is 1200 degrees Fahrenheit; the melting point of zinc is 785 degrees Fahrenheit, and the melting point of tin is 446 degrees Fahrenheit.

I have found in practice that I can obtain a strong, rigid perfect casting, by employing an alloy of 85% zinc, 10% aluminum and 5% tin, which can be poured at about 750° F. to 800° F., the preferred temperature being about 775° F. The pouring temperature may be run up to about 850° F. but this temperature is greater than necessary. If the temperature is too great the overheating will spoil the metal, and, further, the alloy will not run in the mold.

Castings so made run full to the mold, are strong and rigid and there is no breakage due to shrinkage in the mold. The melting point of this alloy can be reduced by increasing the percentage of tin and decreasing the percentage of zinc and alumi-

num and still a good strong casting will result.

While I have given the percentages of zinc, aluminum and tin which I preferably employ, it is of course to be understood these are merely illustrative and that my invention is not to be confined to such percentages.

The alloy should be made by the following method or steps:

The zinc and aluminum are separately melted in separate crucibles or containers. Then the molten aluminum is poured into the molten zinc and stirred thoroughly. Then the molten tin is poured into the combined molten zinc and aluminum and stirred. Among other advantages of this method is that drossing is reduced to a minimum.

Having thus described this invention in connection with illustrative embodiments thereof, to the details of which I do not desire to be limited, what is claimed as new and what is desired to secure by Letters Patent is set forth in the appended claims.

What I claim is:

1. An alloy comprising about 85% of zinc, 10% of aluminum and 5% of tin.
2. A new article of manufacture comprising a strong, rigid and true casting formed of zinc, aluminum and tin, the casting containing about 85% of zinc, about 10% of aluminum and about 5% of tin.
3. The method of manufacturing an alloy of zinc, aluminum and tin consisting in melting the zinc and aluminum separately then pouring one into the other, and then pouring the molten tin into the mixed aluminum and zinc.
4. The method of manufacturing an alloy of zinc, aluminum and tin consisting in separately melting the ingredients, pouring the aluminum into the molten zinc, stirring the mixture thoroughly, and then pouring the molten tin into the mixed molten zinc and aluminum.
5. A metallic alloy adapted for casting, having the characteristics of not shrinking to a material extent in a mold and making a strong, rigid and perfect casting besides being tough and homogeneous, consisting of zinc in largely predominating amount and

containing aluminum and tin each in substantial amounts and containing no substantial amount of other elements.

6. A metallic alloy adapted for casting, having the characteristics of not shrinking to a material extent in a mold and making a strong, rigid and perfect casting besides

being tough and homogeneous and having a relatively low melting point consisting of zinc in largely predominating amount and 10 containing aluminum and tin each in substantial amounts and containing no substantial amount of other elements.

FREDERICK W. KARITZKY.